

Patented Sept. 8, 1925.

1,553,298

# UNITED STATES PATENT OFFICE.

EDWARD C. BURDICK, OF MIDLAND, MICHIGAN, ASSIGNOR TO THE DOW CHEMICAL COMPANY, OF MIDLAND, MICHIGAN, A CORPORATION OF MICHIGAN.

## LIGHT-METAL-CASTING ALLOY.

No Drawing.

Application filed July 12, 1919. Serial No. 310,436.

*To all whom it may concern:*

Be it known that I, EDWARD C. BURDICK, a citizen of the United States, and a resident of Midland, county of Midland, and State of Michigan, have invented a new and useful Improvement in Light-Metal-Casting Alloys, of which the following is a specification, the principle of the invention being herein explained and the best mode in which 10 I have contemplated applying that principle, so as to distinguish it from other inventions.

The present improvements relate more particularly to an alloy in which the metal magnesium largely predominates, in contradistinction to hitherto commercially feasible light metal alloys, in which aluminum has uniformly been the predominant metal. Thus while magnesium has been utilized in 15 combination with aluminum to form the alloy magnalium, all authorities agree that no valuable alloy is produced where the proportion of magnesium exceeds ten per cent, and ordinarily only from one to two per 20 cent of magnesium is utilized in the alloy just referred to.

I have discovered that, contrary to the prevailing understanding, it is possible to produce an alloy of magnesium with aluminum, wherein the former constitutes upwards of ninety per cent of the total mass, which alloy possesses properties admirably adapting it for casting internal combustion motor pistons and other like articles, which 30 require the qualities of lightness, rigidity, and a yield point that is relatively high to the tensile strength. At the same time the alloy which I have obtained is superior for machining, taking a smooth finish at high 35 speeds, without rapid wear of tools, or tearing or pulling along edge of cut. Furthermore, my improved alloy is apparently usable directly without heat treatment, the objectionable tendency to "grow," characteristic of so-called aluminum alloys such as 40 it has heretofore been attempted to use in casting pistons, being so small as to be practically non-existent.

In the production of my improved alloy 50 I employ the ingredients and observe the conditions hereinafter fully set forth and particularly pointed out in the claims, the following description setting forth but one of the several ways in which the principle 55 of the invention may be embodied.

As a result of investigation and experiment, I have found that alloys high in magnesium which, upon cooling, solidify without the formation of a eutectic, lack the rigidity that is not only desirable but necessary in a cast article such as an internal combustion motor piston. In other words, such article will crush under too light a load, and its yield point is relatively low. It is necessary accordingly to add a sufficient quantity of the alloying metal to produce a eutectic, but here again, where the conditions to be met by the cast article when in use involve subjection to a considerable temperature, as in the example of the piston, 60 just referred to, I have found that zinc and other alloy metals which it has heretofore been proposed to use, produce a eutectic of so low a melting point that the composite structure still lacks necessary rigidity and 65 tensile strength.

I have found that a certain limited proportion of aluminum, when added to a predominating quantity of magnesium, goes into solid solution in such magnesium when 70 the mass cools, so that no appreciable eutectic is formed unless upwards of six per cent of aluminum is added. The addition of a further quantity of aluminum, then, 75 will produce a eutectic, and if the amount of such eutectic be not too large the resultant composite structure, consisting of a mass of crystals of solid saturated aluminum-magnesium solution, embedded in and individually more or less surrounded by such 80 eutectic, will possess all of the desired qualities of rigidity, yield point, tensile strength, and workability, specified above. Such alloy will of course be much lighter than one in which aluminum predominates, to a degree 85 corresponding with the relative specific gravities of the two metals.

The most satisfactory proportions of the two metals I have found to be 91.5 per cent of magnesium, and 8.5 per cent of aluminum. Assuming that approximately six per cent of the aluminum goes into the saturated solid solution of the two metals, there is left to go into the eutectic the remaining 2.5 per cent of such metal. I have found that 90 traces—measured in tenths of one per cent—of silicon or of silicon and iron, are of value as apparently additionally contributing to the qualities referred to above. An alloy of the above composition, when cast, 95 100 105 110

has been found to have a yield point of from 12,000 to 14,000 pounds per square inch, and a tensile strength of approximately 20,000 pounds. The co-efficient of expansion, so far as determined, is unexpectedly low, and the cast article may be easily turned or otherwise worked with tools, without dragging or tearing or pulling. The tendency to oxidize, moreover, is no greater, if as great, as in the familiar aluminum alloys, a light coat of the oxide apparently affording complete protection against further action of this sort, while such oxide in the case of the alloy in hand in non-abrasive, which further distinguishes it from the oxide that is formed in the case of such aluminum alloys.

In the case of castings made of the two metals in approximately the proportions indicated above, the structure is found to undergo no appreciable transformation due to alternate heating and cooling, such as internal combustion motor pistons are subjected to. As a result, the objectionable tendency to "grow", which is present even in cast iron pistons, and to an annoying extent in the case of the familiar aluminum alloys, is eliminated. The eutectic formed in the case of an alloy composed of magnesium and aluminum in the proportions stated melts at about 830 degrees F., so that a casting made of such will readily stand temperatures from 700 degrees F. to 800 degrees F. without being affected.

In order to prepare the alloy, the magnesium is first fused in a suitable crucible with a suitable salt flux covering same, and then the measured or weighed amount of aluminum added thereto in the form of small pieces of the solid metal, the mass being thoroughly mixed as such pieces interfuse with the magnesium. The alloy begins to solidify at approximately 1130 degrees F., and while for sand casting it has been found desirable to raise the temperature to from 1200 to 1300 degrees F., a temperature under 1200 degrees is satisfactory for die casting. The flux used to coat the molten metal in the crucible should not be allowed to mingle with the metal that enters the mold in order that the casting may be free from occluded salt or other like impurities.

Other modes of applying the principle of my invention may be employed instead of the one explained, change being made as regards the composition and structure herein disclosed, providing the ingredients or elements of structure stated by any of the following claims or their equivalents be employed.

I therefore point out and distinctly claim as my invention:

1. As a new product, a light metal alloy containing not less than 80 per cent and not more than 99.5 per cent of magnesium, to-

gether with a trace, measured in tenths of one per cent of iron.

2. As a new product, a light metal alloy containing not less than 80 per cent and not more than 99.5 per cent of magnesium, together with a trace, measured in tenths of one per cent of silicon.

3. As a new product, a light metal alloy containing not less than 80 per cent and not more than 99.5 per cent of magnesium, together with traces, measured in tenths of one per cent of iron and silicon.

4. As a new product, a light metal alloy containing magnesium and aluminum wherein the former metal largely predominates, together with a trace, measured in tenths of one per cent of iron.

5. As a new product, a light metal alloy containing magnesium and aluminum wherein the former metal largely predominates, together with a trace, measured in tenths of one per cent of silicon.

6. As a new product, a light metal alloy containing magnesium and aluminum wherein the former metal largely predominates, together with traces, measured in tenths of one per cent of iron and silicon.

7. As a new article of manufacture, a casting made of an alloy of magnesium with aluminum, the latter being present in a quantity not greatly in excess of that required to form a saturated solid solution with the magnesium, and the crystals of such saturated solid aluminum-magnesium solution being uniformly distributed throughout the mass and embedded in a net-work of magnesium-aluminum eutectic so as to produce a finely grained structure.

8. As a new article of manufacture, a casting made of an alloy of magnesium with aluminum, the latter constituting approximately eight and one-half per cent of the total, so as to produce a saturated solid solution with the magnesium with a small excess of aluminum over, and the crystals of such saturated solid aluminum-magnesium solution being uniformly distributed throughout the mass and embedded in a net-work of magnesium-aluminum eutectic so as to produce a finely grained structure.

9. As a new article of manufacture, a casting made of an alloy of magnesium with aluminum, the latter being present in a quantity not greatly in excess of that required to form a saturated solid solution with the magnesium and the crystals of such saturated solid aluminum-magnesium solution being uniformly distributed throughout the mass and embedded in a net-work of magnesium-aluminum eutectic so as to produce a finely grained structure, the casting being substantially free from occluded salt or other like impurities.

10. As a new article of manufacture, a casting made of an alloy of magnesium with

aluminum, the latter constituting approximately eight and one-half per cent of the total, and with a minimum measurable percentage of iron so as to produce a saturated solid solution with the magnesium with a small excess of aluminum over, and the crystals of such saturated solid aluminum-magnesium solution being uniformly distributed throughout the mass and embedded 10 in a net-work of magnesium-aluminum eutectic so as to produce a finely grained structure.

11. As a new article of manufacture, a casting made of an alloy of magnesium with 15 aluminum, the latter constituting approximately eight and one-half per cent of the total, and with minimum measurable percentage of iron and silicon so as to produce a saturated solid solution with the magnesium with a small excess of aluminum over, and the crystals of such saturated solid aluminum-magnesium solution being uniformly distributed throughout the mass and

embedded in a net-work of magnesium-aluminum eutectic so as to produce a finely 25 grained structure.

12. As a new article of manufacture, an internal combustion motor piston casting made of an alloy consisting predominantly of magnesium and containing aluminum in 30 quantity only sufficient to produce a limited amount of eutectic, such aluminum forming with the magnesium a eutectic having a melting point above 700° F., said alloy also containing a trace of iron.

13. As a new article of manufacture, an internal combustion motor piston casting made of an alloy consisting predominantly of magnesium and containing aluminum in 35 quantity only sufficient to produce a limited amount of eutectic, such aluminum forming with the magnesium a eutectic having a melting point above 700° F., said alloy also containing traces of iron and silicon.

Signed by me, this 9th day of July, 1919.  
EDWARD C. BURDICK.